

April 21, 1964

D. M. KOHLER ETAL

3,130,092

PROCESS OF MAKING CUBIC TEXTURE SILICON-IRON

Filed May 29, 1959

3 Sheets-Sheet 1



**FIG. 1.**



**FIG. 2.**



**FIG. 3.**



**FIG. 4.**

INVENTORS.  
DALE M. KOHLER AND  
MARTIN F. LITTMANN,  
BY

*Allen & Allen*

ATTORNEYS.

April 21, 1964

D. M. KOHLER ET AL

3,130,092

PROCESS OF MAKING CUBIC TEXTURE SILICON-IRON

Filed May 29, 1959

3 Sheets-Sheet 2



**FIG. 5.**



**FIG. 6.**



**FIG. 7.**



**FIG. 8.**

INVENTORS.  
DALE M. KOHLER AND  
MARTIN F. LITTMANN,  
BY

*Allen & Allen*

ATTORNEYS.

April 21, 1964

D. M. KOHLER ET AL

3,130,092

PROCESS OF MAKING CUBIC TEXTURE SILICON-IRON

Filed May 29, 1959

3 Sheets-Sheet 3



**FIG. 9.**



**FIG. 11.**



**FIG. 10.**

INVENTORS.  
DALE M. KOHLER AND  
MARTIN F. LITTMANN,  
BY

*Allen & Allen*

ATTORNEYS.

1

3,130,092

PROCESS OF MAKING CUBIC TEXTURE  
SILICON-IRON

Dale M. Kohler, Middletown, and Martin F. Littmann, West Middletown, Ohio, assignors to Armco Steel Corporation, Middletown, Ohio, a corporation of Ohio  
Filed May 29, 1959, Ser. No. 816,889  
9 Claims. (Cl. 148—111)

This is a continuation-in-part of the inventor's copending application of the same title, Serial No. 687,988, filed October 3, 1957, now abandoned.

Silicon-iron sheet stock having a high degree of preferred orientation has come into widespread commercial use, and in many fields the highly directional permeability of such stock has brought about radical changes in the design of transformers and other electrical apparatus. Such silicon-iron products have had a crystal orientation which may be designated as (110)[001] in the standard notation of Miller's indices. This orientation means that the product has a high permeability in the rolling or "straight-grain" direction, but a poor permeability in other directions.

The crystalline structure of silicon-iron is cubic, so that the individual crystals in a polycrystalline material may be visualized as a series of cubes. In the orientation mentioned above, a cube edge [001] is parallel to the rolling direction and a dodecahedral face (110) is parallel to the rolling plane. Four of the cube edges are parallel to the direction of rolling, but no face of the cube is parallel to the surfaces of the sheet. Thus, the orientation has been referred to as a "cube-on-edge" type. The cube edges which lie transverse to the direction of rolling are not parallel to the surfaces of the sheet. Consequently, the transverse permeability is low because the most effective path for the magnetic flux, is parallel to the cube edges.

It has been realized that if it were possible to so orient the crystals that while a cube edge remained parallel to the rolling direction, another cube edge would lie perpendicular to the rolling direction and in the plane of the sheet surface, a material would be obtained which not only would have a high straight grain permeability but would also have a high transverse or "cross grain" permeability. Such a product would have many additional uses, particularly in the construction of transformers having cores made from E or I-shaped laminations and in rotating electrical machinery. The orientation just described is a (100)[001] orientation by Miller's indices and for convenience hereinafter will be referred to by the arbitrary expression "cubic texture."

Hitherto it has not been possible to attain a cubic texture with commercial reproducibility and at commercial cost by starting with a polycrystalline silicon-iron and orienting the crystals therein by a combination of cold reductions and heat treatments. It is a primary object of this invention to provide such a process.

It is an object of the invention to provide an oriented product of polycrystalline character having more than one direction of high permeability.

It has been noted that as silicon-iron having the cube-on-edge type of orientation becomes thinner, the hysteresis loss of the material increases sharply, probably because of the increased effect of the unfavorable crystallographic directions which lie in the plane of the sheet. It is an object of this invention to provide a polycrystalline silicon-iron which minimizes this defect.

The attaining of a high degree of cubic texture in silicon-iron is accomplished by secondary recrystallization of a material characterized by some grains which are already in the desired orientation (or within a comparatively few degrees of it), which grains or nuclei

2

grow during the secondary recrystallization at the expense of grains having a substantially different orientation.

It is an object of this invention to provide a method of making a material, and a material so made, which can be depended upon to have a comparatively large number of nuclei in or near the (100)[001] orientation and a minimal number of grains in other orientations which might also tend to grow during secondary recrystallization at the expense of grains having substantially different orientations.

These and other objects of the invention which will be set forth hereinafter or will be apparent to one skilled in the art upon reading these specifications are accomplished in that procedure and product of which an exemplary embodiment will hereinafter be described. Reference is made to the accompanying drawings wherein:

FIG. 1 is a stereogram of the cube poles of representative individual grains of a silicon-iron piece characterized by the cube-on-edge type of orientation.

FIG. 2 is a diagrammatic representation of this type of orientation.

FIG. 3 is an X-ray pole-density stereogram of (200) poles showing a derivative orientation designatable as (111)[112], produced by cold rolling the material of FIG. 1.

FIG. 4 is a diagram of this type of orientation.

FIG. 5 is an X-ray pole-density stereogram of (200) poles showing a derivative orientation which may be designated as (120)[001], resulting from the recrystallization of the product of FIG. 3.

FIG. 6 is a diagram of this type of orientation.

FIG. 7 is an X-ray pole-density stereogram of (200) poles of material showing a derivative orientation (hereinafter described) produced by another stage of cold rolling.

FIG. 8 is a diagram of this orientation.

FIG. 9 is an X-ray pole-density stereogram of (200) poles of the material of FIG. 7 after a primary recrystallization.

FIG. 10 is a stereogram of the cube poles of individual grains of the material of FIG. 9 after having been subjected to secondary recrystallization, and showing cubic texture, designatable as (100)[001].

FIG. 11 is a diagram of this orientation.

On the X-ray pole-density stereograms, FIGS. 3, 5, 7 and 9, numerical indications of the intensities are shown in "times random."

The silicon-iron material employed in the practice of the invention should have a silicon content sufficiently high to prevent phase changes during heat treatment, but low enough to prevent brittleness during rolling. A range of 2.5 to 4.0% silicon is satisfactory. The final product should have a high degree of purity by which is meant freedom from carbon, sulphur, nitrogen, oxygen, inclusions and the like. Purity is usually attained in the production of the metal in known ways, although carbon may be reduced at any early heat treating stage of the routing by subjecting the material to a decarburizing anneal, preferably in accordance with the teachings of the Carpenter et al. Patent No. 2,287,467, issued June 23, 1942.

By way of example, a preferred range of silicon is from 2.90 to 3.30%. The cube-on-edge material should contain .007% or less carbon, .03 to .15 manganese, and .015 to .030% sulfur, the remainder being substantially all iron with normal impurities, and with a total oxide content of .015% or less.

The low carbon content is important because it makes for low core loss values. The total oxide content is preferably no more than .004% in the final product just before secondary recrystallization.

Hot rolled silicon-iron is generally characterized by an

incompletely developed preferred crystal orientation. In both hot and cold rolling, the crystals not only become longer but tend to change their orientation by a process of slip in preferred directions and on preferred crystallographic planes. In this manner, deformation produces a preferred texture in the material, with the individual crystals in various conditions of stress. Raising the temperature after deformation permits the crystals to release their stresses through recrystallization; and the crystals generally change in orientation by the adoption of adjacent positions of lower energy.

The art has hitherto learned various procedures for producing from polycrystalline silicon-iron the material above designated as of the cube-on-edge type, by subjecting the hot rolled material to one or to a series of controlled cold reductions followed by heat treatments. Our researches have indicated that the cube-on-edge or (110)[001] orientation is in many instances at least a derivative of a (111)[112] orientation produced by tilting the crystals in the rolling direction by a sufficient amount and then causing them to assume a related low energy position which is the cube-on-edge orientation. As examples of suitable procedures, reference may be made to Patent 2,158,065, dated May 16, 1939, in the names of Cole et al., Patent 2,287,466, dated June 23, 1942, in the name of Carpenter, Patent 2,307,391, dated January 5, 1943, in the names of Cole et al., and Patent 2,599,340, dated June 3, 1952, in the names of Littmann et al. FIG. 1 of this application is a stereogram of the cube poles of typical cube-on-edge silicon-iron, clearly indicated in a crystal position such as is illustrated in FIG. 2 hereof. In this figure two small cubes 1 and 2 have been shown, the rolling direction being indicated by an arrow, and the planes of the surfaces of the sheet material being understood to be parallel to the plane of the paper on which the drawing is made.

It has now been discovered that it is possible to take commercial polycrystalline silicon-iron having the (100)-[001] orientation and convert it to a polycrystalline material having the (100)[001] orientation or cubic texture by a series of progressive steps. Material suitable for this process consists of sheet or strip of any thickness having a cube-on-edge orientation as illustrated in FIGS. 1 and 2, prepared in any suitable way including the procedures of the above mentioned patents.

It will be understood that the commercial starting material will have purity within the limits set forth above, will have been decarburized to the desired degree, and will have been subjected to a "final" heat treatment at high temperature (generally around 2200° F.).

The first step is to cold reduce such material within certain limits so as to bring about the tilted condition of the crystals indicated in the pole-density stereogram which forms FIG. 3 hereof and illustrated by the small cubes 3 and 4 of FIG. 4. A cold reduction generally of about 55% to 90% will produce the effect, it being understood that the tilting will vary with the degree of cold rolling reduction. The orientation at this stage will respond generally to the notation (111)[112] of Miller's indices.

It has been found that the optimum ranges for cold rolling in the first stage just described differ depending upon whether the immediate anneal which follows is an open anneal or a box anneal. If the anneal is an open anneal, best results will be obtained if the reduction is about 75% to 87%. If a box anneal is used at this point, best results will be attained at reductions of about 60% to 85%.

The material is next subjected to an intermediate anneal in which primary recrystallization occurs. The texture or orientation which results is illustrated in the pole figure which is FIG. 5 of the drawing, and which is diagrammed in FIG. 6 at 5 and 6. It is an orientation which can be described as having a cube edge in the rolling direction and having a cube face rotated 22½°

each way about the rolling direction from the rolling plane. While some variation in this texture can be tolerated, it is preferable to have the crystals preponderantly with their (120) planes in substantial parallelism with the planes of the sheet material.

The intermediate anneal which accomplishes this is an anneal, either open or box, preferably at about 1200° to 2200° F., and preferably in dry hydrogen. If an open or strip anneal is used, a temperature of 1500° to 1700° F. is preferred. If a box anneal is used, a preferred range is 1400° to 1600° F., although good results may be obtained over the entire range given above, namely 1200° to 2200° F. The annealing atmosphere should be such as to preclude undue oxidation.

The material is next subjected to a second cold rolling treatment. In the cold reduction the crystals are again tilted, and this produces the complex pole density stereogram which forms FIG. 7 hereof. A study of this stereogram will indicate that the orientation of the crystals is substantially that diagrammed at 7, 8, 9 and 10 in FIG. 8. The crystal orientation illustrated is obtained by rotating the cubes substantially 30° each way about the transverse axis, and then substantially 10° about an axis normal to the sheet surface. If this index were to be described by the use of Miller's indices, It would approximate a (7,10,15)[13,6,10] orientation.

Again to produce this orientation the cold rolling treatment must be controlled as to extent. A cold rolling reduction of about 50% to 80% will generally be found effective. This second cold rolling is, however, affected by the nature of the intermediate anneal previously outlined. Thus if the intermediate anneal is an open or strip anneal an optimum range of reduction in the second cold rolling treatment will be found to be about 60% to 70%. If a box anneal has been practiced, a percentage reduction in the second stage of cold rolling of a somewhat higher value, namely 70% to 80% will be found best.

A material oriented as shown in FIGS. 7 and 8 can be caused to assume the orientation indicated by the pole density stereogram set forth here as FIG. 9, by primary recrystallization. An examination of this stereogram will indicate that while the cube edges have been realigned in the rolling direction with reasonable uniformity, the tilting of the cube faces with reference to the plane of the sheet stock has broadened and becomes more heterogeneous. A large number of the grains are tilted by more than 22½° from the position illustrated in FIG. 6 as the (120)[001] orientation, and a substantial number have been tilted into the (100)[001] position or within a few degrees of it. It is these last mentioned grains which form the nuclei for the subsequent conversion of the stock to one having preponderantly the cubic orientation, in the process of secondary recrystallization.

The skilled worker in the art will understand that primary recrystallization occurs rapidly at a relatively lower temperature, in the range of say 1075° to 1900° F., while secondary recrystallization requires time at a higher temperature of about 1900° to 2300° F., with a preferred temperature at about 2200° F. Consequently after the last cold rolling treatment, the primary and secondary recrystallizations are usually carried on in a single heat treatment under conditions hereinafter to be specified.

As in other procedures for the production of highly oriented silicon-irons involving a series of cold reductions which are critical as to amount, it will be necessary to calculate back from the finished gauge in order to determine the proper thickness of the starting material. Beyond this there is no limit on the present invention either as to the thickness of the final product or as to the thickness of the starting material.

The original material is, of course, an ingot of silicon-iron alloy which may be processed into suitable cube-on-edge sheet or strip material in a variety of ways as has

been described heretofore. The cube-on-edge stock which forms the starting material here should have a high degree of perfection of the (110)[001] orientation. The term high degree should be taken as indicating that the material is so oriented as to have a straight grain permeability of at least about 1700 at  $H=10$  oersteds, and preferably higher. The cube-on-edge material preferably has a relatively large grain size (about 5 mm. in diameter).

In the next stage of the process, the material having the high degree of (110)[001] orientation is cold reduced to a thickness of about  $\frac{1}{2}$  to  $\frac{1}{10}$  its original thickness, i.e., with a reduction of 55% to 90%, or within the narrower preferred ranges discussed above. It is then recrystallized. Varying heat treatments at this point are possible. An open, strand or continuous anneal may be used; but a box anneal in an inert or reducing atmosphere such as hydrogen is preferred. The material may be heated to a temperature of about 1200° to 2200° F. and held for about two hours at such temperature. Assuming the product has the desired purity and has previously been decarburized to, say, .01% or lower, the essentials here are to effect a primary recrystallization and fit the material for further cold reduction, while avoiding the development of oxides at its surfaces.

Next the product having the high degree of (120)[001] orientation is again cold reduced to about  $\frac{1}{2}$  to  $\frac{1}{5}$  its thickness or with a reduction of 50% to 80%, or preferably within the narrower preferred ranges discussed above.

The final rolled product is then given a box anneal in hydrogen. While the attainment of a recrystallizing temperature will produce a substantial number of grains having the desired (100)[001] orientation if the preceding steps have been performed, a product in which at least the majority of the grains have the (100)[001] orientation is obtained when discontinuous or selective grain growth takes place. This grain growth, sometimes called "secondary recrystallization," takes place at temperatures above about 1900° F. To promote secondary grain growth the annealing atmosphere should be pure and non-reactive. Annealing separators may be used. While hydrogen is suitable, the use of vacuum or inert atmospheres like helium, argon or the like is desirable. In the secondary recrystallization, the (100)[001] crystals tend to grow at the expense of the other crystals, producing a very nearly perfect orientation in the cubic texture.

The final heat treatment is preferably carried on in accordance with the teachings of the copending application of Kohler (one of the inventors herein) entitled The Production of Oriented Silicon-Iron Sheets by Secondary Recrystallization, Serial No. 813,289, filed May 14, 1959, which teaches in essence the use of an atmosphere in the final heat treatment of hydrogen or a non-reactive gas such as argon or helium, which atmosphere contains a very small amount of a highly polar compound such as hydrogen sulphide, sulphur dioxide, an oxide of carbon, or a mixture of these. The highly polar compound is believed to be absorbed or adsorbed on the crystal planes at the surfaces of the sheet stock so as to satisfy the positive unsatisfied charges there, the result being a shifting of the energies of crystals of differing orientations in such a way that the (100)[001] orientation becomes the lowest energy orientation by a substantial amount, making for a more positive and complete cubic texture orientation in the stock.

The final anneal may be and preferably is a box anneal, although it has been found that an open, strand or continuous anneal may be used.

The result of the final anneal is illustrated by the stereogram FIG. 10, and diagrammed in FIG. 11. It has been found readily possible in accordance with the teachings of this application to make a silicon-iron product in which in excess of 90% of the surface area of the sheet stock is occupied by grains having the cubic tex-

ture, the grains nevertheless being comparatively small, which is favorable to core loss characteristics. A grain size of 7 (ASTM) at 1 $\times$  magnification or smaller can be produced especially if box annealing treatments are employed.

#### Example

A coil of silicon-iron .014 inch in thickness, containing 3% silicon, and already having the (110)[001] orientation was selected. This material had a permeability at  $H=10$  of about 1820 in the straight grain direction, and the orientation shown in FIG. 1. It had a grain size of about 7 in accordance with the ASTM standards at 1 $\times$  magnification, after hydrogen annealing for 24 hours at 2200° F. This coil was pickled and cold reduced to .0038 inch and exhibited the orientation shown in FIG. 3. The strip was then strand annealed in hydrogen for 2 minutes at 1600° F. It now had the (120)[001] texture shown in FIG. 5.

The material was then again cold rolled to a thickness of .0018 inch. Its orientation at this stage is shown in FIG. 7.

Finally, the material after shearing into Epstein samples (3 cm. x 30.5 cm.), samples being taken both in the rolling direction and transverse it, was given an anneal in hydrogen, the heating cycle being such that it took the material about 8 hours to attain a temperature of 2200° F. It was held at this temperature for about 5 hours.

Examination of the surface of the final product indicated that at least about 90% of its area was occupied by crystals which were the product of secondary crystal growth. FIG. 10 is the X-ray pole figure of the product. The product tested as follows:

Permeability at  $H=10$  oersteds, 1840 (straight grain)  
Permeability at  $H=10$  oersteds, 1780 (cross grain)

Modifications may be made in the invention without departing from the spirit of it. The invention having been described in an exemplary embodiment, what is claimed as new and desired to be secured by Letters Patent is:

1. A process of producing silicon-iron for magnetic uses having high straight-grain and high cross-grain permeabilities, which comprises providing a polycrystalline ferrous sheet stock containing substantially 2.5 to 4.0% silicon and having preponderantly a (100)[001] crystal orientation by Miller's indices, cold rolling said silicon-iron with a reduction of substantially 55 to 90%, and subjecting said silicon-iron to a primary recrystallization in a heat treatment at about 1200° F. to 2200° F., then again cold rolling said silicon-iron with a reduction of substantially 50% to 80%, and heat treating the silicon-iron at a temperature of 1900° to 2300° F. under conditions productive of secondary recrystallization whereby first to subject said silicon-iron to primary recrystallization, and thereafter to secondary recrystallization to convert said silicon-iron to a polycrystalline product having preponderantly a (100)[001] orientation.

2. A process of producing silicon-iron for magnetic uses having high straight-grain and high cross-grain permeabilities, which comprises providing a polycrystalline silicon-iron containing substantially 2.5 to 4.0% silicon having preponderantly a (110)[001] crystal orientation by Miller's indices, cold rolling said silicon-iron with a reduction of substantially 55 to 90%, whereby to convert it to a material having a (111)[112] orientation, subjecting said silicon-iron to a heat treatment at above the recrystallization temperature whereby to convert the orientation to (120)[001], again cold rolling said silicon-iron with a reduction of substantially 50 to 80% to convert the last mentioned orientation to a derivative orientation in which the crystals are tilted in both transverse directions as respects the rolling direction, and subjecting said silicon-iron to a heat treatment at about 1900° to 2300° F. under conditions productive of sec-

ondary recrystallization, whereby to effect a primary recrystallization followed by a secondary recrystallization.

3. The process claimed in claim 2 wherein the starting material has a straight-grain permeability of at least about 1700 at  $H=10$ .

4. A process of producing silicon-iron sheet stock for magnetic uses having high straight-grain and high cross-grain permeabilities, which comprises hot rolling an ingot of silicon-iron containing substantially 2.5 to 4.0% silicon, converting it by at least one cold rolling treatment followed by a recrystallization to a (110)[001] orientation with a straight-grain permeability of at least about 1700 at a magnetizing force of 10 oersteds, converting it by an additional cold rolling treatment with substantially 55 to 90% reduction and a primary recrystallizing heat treatment through a (111)[112] orientation to preponderantly a (120)[001] orientation, and converting it by a cold rolling reduction of substantially 50 to 80% and a primary recrystallizing heat treatment through a derivative cold rolled orientation in which the (120)[001] crystals are tilted in both transverse directions as respects the rolling direction, to an orientation in which the cube edges are generally aligned in the rolling direction but the cube faces are tilted away from the (110) position, the said tilting being such that a substantial number of the grains have their cube faces substantially parallel to the faces of the sheet stock, and then subjecting the stock to a secondary recrystallization to cause said last mentioned grains to grow, until the greater part of the face area of said sheet stock is occupied by grains having a (100)[001] orientation.

5. The process claimed in claim 4 in which the said final heat treatment carries the said silicon-iron to a temperature of at least substantially 2000° F. and includes a soaking at the said temperature, whereby said secondary recrystallization is caused to take place.

6. A process of making cubic texture silicon-iron sheet stock containing substantially 2.5% to 4.0% silicon which comprises providing a silicon-iron sheet stock the grains of which are characterized by a (110)[001] orientation, cold rolling said stock with a reduction of substantially 55% to 90% reduction, annealing said stock at a temperature of substantially 1200 to 2200° F., again cold rolling said stock with a reduction of substantially

50% to 80%, subjecting said stock to a primary recrystallization at a temperature of substantially 1075° to 1900° F., and then to a secondary recrystallization at a temperature of substantially 1900° to 2300° F.

5 7. The process claimed in claim 6 in which said secondary recrystallization is carried on in a non-oxidizing atmosphere containing a minute quantity of polar compound chosen from a class consisting of oxides of sulfur and carbon and hydrogen sulfide.

10 8. A process of making cubic texture silicon-iron sheet stock containing substantially 2.5% to 4.0% silicon, which comprises providing a silicon-iron sheet stock the grains of which are characterized by a (110)[001] orientation, cold rolling said stock with a reduction of substantially 75% to 87%, strip-annealing said stock at a temperature of substantially 1500° to 1700° F., again cold rolling said stock with a reduction of substantially 60% to 70%, subjecting said stock to a primary recrystallization at a temperature of substantially 1400° to 1700° F., and to a secondary recrystallization at a temperature of substantially 190° to 2300° F.

15 9. A process of making cubic texture silicon-iron sheet stock containing substantially 2.5% to 4.0% silicon, which comprises providing a silicon-iron sheet stock the grains of which are characterized by a (110)[001] orientation, cold rolling said stock with a reduction of substantially 60% to 85%, box annealing said stock at a temperature of substantially 1400° to 1600° F., again cold rolling with a reduction of 70% to 80%, and then subjecting said stock to a primary recrystallization and a secondary recrystallization in a box anneal at a temperature of substantially 1900° to 2300° F.

References Cited in the file of this patent

UNITED STATES PATENTS

|           |               |               |
|-----------|---------------|---------------|
| 2,473,156 | Littmann      | June 14, 1949 |
| 2,867,558 | May           | Jan. 6, 1959  |
| 2,992,951 | Aspden        | July 18, 1961 |
| 2,992,952 | Assmus et al. | July 18, 1961 |

FOREIGN PATENTS

|           |         |              |
|-----------|---------|--------------|
| 1,009,214 | Germany | May 29, 1957 |
|-----------|---------|--------------|

UNITED STATES PATENT OFFICE  
CERTIFICATE OF CORRECTION

Patent No. 3,130,092

April 21, 1964

Dale M. Kohler et al.

It is hereby certified that error appears in the above numbered patent requiring correction and that the said Letters Patent should read as corrected below.

Column 3, line 38, and column 6, line 46, for "(100)", each occurrence, read -- (110) --; column 4, line 26, for "10" read -- 10 --.

Signed and sealed this 8th day of September 1964.

(SEAL)

Attest:

ERNEST W. SWIDER  
Attesting Officer

EDWARD J. BRENNER  
Commissioner of Patents